

## UNITED STATES PATENT OFFICE

1,938,015

IMITATION RUBBER AND PROCESS OF  
MANUFACTURING THE SAMEShozo Fuji and Tatsuzo Fukuda, Utsunomiya-  
Shi, JapanNo Drawing. Application May 15, 1931  
Serial No. 537,750

2 Claims. (Cl. 106—23)

This invention has relation to the manufacture or production of imitation rubber from vegetable oils by the action of lead salts and the object of the invention is to produce a lead salt of fatty acid in the form of a liquid of viscous character having the properties to a certain extent of natural rubber and which may be used as a substitute therefor in many industries, being, when dry, flexible, elastic and transparent also insoluble in dilute mineral salts or fatty acids, and being also waterproof.

In carrying our invention into effect, we heat a vegetable oil such as the oil of perilla coimoides to 250° C., stirring the same strongly and we then add slowly 5-10% of lead carbonate and then heat them step by step to 300° C., and after being stirred for about thirty minutes in the same condition, carbonic acid gas escapes therefrom as bubbles.

When the mixtures have been allowed to cool to 200° C., there appears a yellowish brown viscous liquid on the surface in which lead salts of fatty acids are the main components.

This liquid consists of different formations by the quantity of lead salt, and there may be derived various viscous liquids by the process. Several liquids can be obtained for use in painting upon paper or cloth. The liquid will permeate the material to which it is applied, and when the material is dried in the air the liquid absorbs oxygen and solidifies, thus producing the required film.

This imitation rubber, or rubber substitute is

elastic and flexible yet will not dissolve in dilute mineral salts or fatty solvents.

Shiny films, are produced, which are heat proof and water proof and are similar to natural rubber in external appearance and to the sense of touch and will not harden or slacken under changes in temperature.

The liquid material when painted on the surface of metal or wood is stainless and anti-septical and also when painted on the surface of cloth has the effect of protecting the same from moisture.

We claim:

1. The process for the production of imitation rubber, which consists in heating a vegetable oil, such as perilla, to a temperature of about 250° C., stirring the same and adding thereto 5-10% of lead carbonate, heating the mixture gradually to a temperature of about 300° C. and continuing the heating at this temperature, until the lead carbonate decomposes, liberating carbonic acid gas, and at the same time combining with part of the oil to form a lead salt of the oil, whereby a rubber-like material is obtained.

2. A viscous rubber like product resulting from the reaction of 5 to 10% of lead carbonate on a vegetable oil, which product, on exposure to air, congeals, is flexible and transparent and is insoluble in water, fatty acids or dilute mineral salts.

SHOZO FUJI.  
TATSUZO FUKUDA.

35

90

40

95

45

100

50

105

55

110